# EUROPEAN PATENT APPLICATION

(11) **EP 2 006 419 A1**
(43) Date of publication of application: **24.12.2008**
(21) Application number: 07110910.2
(22) Date of filing: 22.06.2007
(51) Int. Cl.: C25C 3/12, C25C 3/16

(54) **Reduced voltage drop anode assembly for aluminium electrolysis cell**

(71) Applicant: SGL Carbon AG, 65203 Wiesbaden (DE)
(72) Inventor: Hiltmann, Frank, 65830, Kriftel (DE); Christ, Martin, 86159, Augsburg (DE); Langer, Werner, 86450, Altenmünster (DE); Öttinger, Oswin, 86405, Meitingen (DE)

(57) **Abstract**

Anode assembly for aluminium electrolysis cells comprising carbon anodes (2) with stubholes (5) and an anode hanger having stubs (4), whereas the anodes (2) are fixed to the anode hanger by cast iron (6), characterized in that the stubholes (5) are fully or partially lined with an expanded graphite lining (7).
Such anode assemblies provide reduced voltage drop across the interface between the cast iron (6) and the carbon anode (7) and thus increase cell productivity significantly. Further, mechanical stresses in the stubhole (5) area are reduced. By further forming a collar (8) from the lining (7), the spilling of cast iron over the anode (2) surface is prevented and optionally a protective shot plug or a protective collar prevent direct contact of the hot electrolyte bath with the stub (4) and the cast iron (6).

## Description

The invention relates to anode assemblies for aluminium electrolysis cells consisting of carbon anode blocks and anode hangers attached to those blocks whereas the anode stubholes receiving the anode hanger stubs are lined with expanded graphite. As a consequence, the contact resistance between anode block and cast iron sealant is reduced resulting in a reduced voltage drop across this interface. Further, the expanded graphite lining may form a collar providing additional benefits of this invention.

Aluminium is conventionally produced by the Hall-Heroult process, by the electrolysis of alumina dissolved in cryolite-based molten electrolytes at temperatures up to around 970 °C. Hall-Heroult aluminum reduction cells are operated at low voltages (e.g. 4-5 V) and high electrical currents (e.g. 100,000-350,000 A). The high electrical current enters the reduction cell from the top through the anode structure and then passes through the cryolite bath, through a molten aluminum metal pad, enters the carbon cathode block, and then is carried out of the cell by the collector bars.

A Hall-Heroult reduction cell typically has a steel shell provided with an insulating lining of refractory material, which in turn has a lining of carbon contacting the molten constituents. Steel-made collector bars connected to the negative pole of a direct current source are embedded in the carbon cathode substrate forming the cell bottom floor.

One or more carbon anode blocks are provided above each cathode block and are partly submerged in the cryolite bath. The carbon anodes are manufactured by mixing petroleum coke and pitch, forming the mixture into blocks including stubholes for the electrical connection, and subsequently baking them.

In an electrolysis cell of common size there are about 20-30 carbon anodes, and since these anodes are consumed gradually, they have to be changed ususally within a month, depending on the size of the anodes and amperage applied. Thus, in each cell there is one anode exchanged every day.

The carbon anodes are fixedly connected to anode hangers. The anode hangers serve two different purposes, namely to keep the carbon anodes at a predetermined distance from the cathode, and to conduct the electric current from an anode bar down through the carbon anodes. The anode hangers are fixed to an overhanging anode bar by means of a clamping device in a detachable manner. As the carbon anodes are gradually consumed and as aluminium metal is removed from the cells, the anode bar, with the carbon anodes attached thereto, is lowered to keep a constant distance between the bottom side of the anodes and the aluminium pad. As cell amperage is very high, electric current connections and bus bars are therefore made of industrial metals with good electric conductivity i.e. usually pure copper or aluminium.

Since the lower part of the anode hangers is situated close to the cryolite bath which is of a high temperature, this part of the anode hanger is made of material which is resistant to the high temperature, usually steel.

An anode hanger consists of aluminium or copper rods welded or bolted to steel stubs. To produce an anode assembly, the cylindrical stubs of the anode hanger are then positioned in the pre-formed conical stubholes of the anodes and molten cast iron is poured around the stubs (called "rodding").

The voltage drop between stub and carbon anode is an essential part of the overall voltage drop at the anode and has a detrimental impact on the electrolytic process.

The Ohmic heat, which is generated due to a high voltage drop at the anode has a strong thermal effect on the electrolytic bath, and should be minimized. The less heat is evolved in the anode, the more heat can be generated in the electrolyte. This allows an increase in anode-cathode distance (ACD), which in turn is favorable when aiming at boosting of current density as well as current efficiency. As practical measurements have shown, the stub-to-anode voltage drop is of the same order of magnitude as the average voltage drop in the anode block itself. This effect is even more remarked when a new anode assembly has just been put in operation. This effect can be attributed to the different thermal expansion coefficients of the steel stub, cast iron and carbon anode.

It was therefore concluded that the potential in reducing the voltage drop between stub and carbon anode is greater than in the carbon anode itself.

This problem has been partially addressed in the prior art. For example, German Pat. DE 1 187 807 discloses a carbon anode having one or more cavities to receive a metal stub or rod. The surfaces of the cavities have grooves or teeth to increase the surface area which is said to provide better conductivity of the current from the rod into the anode.

Russian Pat. No. 378,524 illustrates a carbon electrode structure having the usual central stubhole to receive a metal stub and also having a series of stubholes drilled into the carbon block parallel to the central stubhole to receive cast iron rods. Openings are then cut into the carbon between the central stubhole and the cast iron rods to permit cast iron bridge pieces to be poured to connect the cast iron rods to the metal stub.

The above attempts do provide for a more even current distribution across the upper part of the anode block but require substantial adjustments to the anode as well as stub design and further do not address the substantial voltage losses at the stub-anode-interface.

It is therefore an object of the present invention, to provide anode assemblies comprising carbon anode blocks with stubholes being attached to an anode hanger, characterized by the stubholes are lined fully or partially with expanded graphite. Expanded graphite (EG) provides a good electrical and thermal conductivity especially with its plane layer. It also provides some softness and a good resilience making it a common material for gasket applications. Those characteristics render it an ideal material to improve the contact resistance between the anode block and the cast iron. The resilience also significantly slows down the increase of contact voltage drop at the interface between cast iron and anode blocks during electrolysis as it can fill out the gaps formed due to creep of the involved materials. Increase of contact voltage drop at the interface between cast iron and anode blocks is further reduced especially by the EG lining at the bottom of the anode stubhole as it acts as barrier to e.g. aluminium diffusing through the anode block, thus preventing formation of insulating layers at said interface.

Further, the resilience of EG eases mechanical stress due to different coefficients of thermal expansion between steel stub, cast iron and anode block. Thermal expansion of the different materials occurs mainly during pre-operational heating-up of the electrolysis cell and also during rodding and frequently results in cracks in the anode block that further reduce their lifetime.

The invention will now be described in more detail with reference to the accompanying drawings in which:
Figure 1 shows an anode hanger onto which is mounted a carbon anode,
Figure 2 shows an enlarged section of the prior art connection between a stub and the carbon anode,
Figure 3 shows an enlarged section of the connection according to this invention between a stub and the carbon anode,
Figures 4 to 6 show an enlarged section of the connection according to this invention between a stub and the carbon anode, whereas the expanded graphite lining extends above the stubhole thus forming a collar
Fig. 7 shows a schematic sketch of the laboratory test setup for testing the change of contact resistance at the stub-to-anode interface

Fig. 1 shows an anode assembly 1 with an anode hanger 3 supporting a carbon anode 2 which is used in cells producing aluminium by electrolysis. The three downwardly protruding steel stubs 4 of the anode hanger are extending each into the stubholes 5 of the anode 2 and are fixed there by pouring cast iron 6 into the gap formed between the stub 4 and the anode 2 as shown in Fig. 2.

Fig. 3 shows an anode-stub-connection according to this invention. The stubhole 5 of the anode 2 is lined with an expanded graphite lining 7 and the gap between the lining 7 and the anode stub 4 is filled with cast iron 6.

The lining 7 may be applied to the entire surface of stubhole 5. Further, lining 7 may only be applied to parts of the surface of stubhole 5.

The expanded graphite lining 7 is preferably provided as thin foil but can also be provided by coating the stubhole 5 with a paste consisting of expanded graphite and a hardenable binder, such as phenolic resin. In the latter case, the cast iron 6 is preferably poured into the lined stubhole 5 after the binder has cured. If the lining 7 consists of graphite foil, it can be attached to the stubhole 5 surface with a glue. A further advantage of this invention is that the graphite foil may be pre-shaped as sleeve or socket prior to the lining to simplify the lining process.

The thickness and density of lining 7 depends largely on the stubhole 5 dimensions and operational parameters. In addition to the reduction of the contact resistance, the expanded graphite lining 7 also acts as a barrier against chemical compounds diffusing through the anode 2 block towards the cast iron 6. It also buffers thermomechanical stresses, depending on the specific characteristics of the selected expanded graphite quality.

Further, if lining 7 is based on graphite foil, it may preferably extend above the stubhole 5, thus forming a small collar 8. The collar 8 prevents cast iron 6 to be spilled over the anode 2 surface during casting. In this manner, the used anodes 2 can be more easily detached from the stubs 5 after operational life in the cell.

According to another embodiment of this invention, a protecting ring can be formed by filling the free space of the collar 8 above the cast iron 6 carbonaceous paste 9 and finally hardening this paste to form a protective shot plug. This measure prevents the electrolytic bath from coming into contact with the steel stub 5 and the cast iron 6. According to yet another embodiment of this invention as shown in Fig. 6, the sleeves of the expanded graphite collar 8 above the cast iron 6 are simply bent downwards to the stubhole 4 thus forming a protective collar. This measure prevents the electrolytic bath from coming into contact with the steel stub 5 and the cast iron 6.

The contact resistance between the stub and the carbon anode was determined with a laboratory test device depicted in Fig. 7. The device measured the change of through-plane resistance under load. This test setup was used to mimic the effects of using expanded graphite lining 7 for lining the stubholes 5. Various types and thicknesses of expanded graphite foil (for example SIGRAFLEX F02012Z) have been tested using loading/ unloading cycles. Specimen size was 25mm in diameter. The tests were carried out using an universal testing machine (FRANK PRÜFGERÄTE GmbH). The anode specimen were manufactured in following manner. 100 parts petrol coke with a grain size from 12 µm to 7 mm were mixed with 25 parts pitch at 150 °C in a blade mixer for 10 minutes. The resulting mass was extruded to a blocks of the dimensions 700 x 500 x 3400 mm (width x height x length). These so-called green blocks were placed in a ring furnace, covered by metallurgical coke and heated to 900 °C. Afterwards small specimen pieces were cut from the block.

A comparison of the test curves revealed significant decrease (by over 20%) in through-plane resistance especially at lower loadings by the inventive system with expanded graphite. This advantage is also maintained upon load relaxation due to the resilience of the expanded graphite.

It was thus shown that the here described invention can significantly contribute to lowering the voltage drop at the anodes 2 of aluminium electrolysis cells.

Having thus described the presently preferred embodiments of our invention, it is to be understood that the invention may be otherwise embodied without departing from the spirit and scope of the following claims.

### Key to figures:

(1) anode assembly
(2) carbon anode
(3) anode hanger
(4) anode hanger stub
(5) anode stubhole
(6) cast iron
(7) expanded graphite lining
(8) collar formed by expanded graphite lining
(9) carbonaceous paste

## Claims

1. Anode assembly 1 for aluminium electrolysis cells comprising carbon anodes 2 with stubholes 5 and an anode hanger 3 having stubs 4, whereas the anodes 2 are fixed to the anode hanger 3 by cast iron 6, **characterized in that** the stubholes 5 are fully or partially lined with an expanded graphite lining 7.

2. Anode assembly 1 according to claim 1, **characterized in that** the expanded graphite lining 7 consists of graphite foil.

3. Anode assembly 1 according to claim 2, **characterized in that** the expanded the graphite foil is pre-shaped as sleeve or socket.

4. Anode assembly 1 according to claim 1, the expanded graphite lining 7 consists of a paste consisting of expanded graphite and a hardenable binder, such as phenolic resin.

5. Anode assembly 1 according to claims 2 or 3, **characterized in that** the expanded graphite lining 7 extends above the stubhole 5 to form a collar 8.

6. Anode assembly 1 according to claim 5, **characterized in that** the free space within the collar 8 above the cast iron 6 is filled with carbonaceous paste 9.

7. Anode assembly 1 according to claim 5, **characterized in that** the sleeves of the expanded graphite collar 8 above the cast iron 6 are bent downwards to the stubhole 4 to form a protective collar.

8. Method of manufacturing anode assemblies 1 for aluminium electrolysis cells, **characterized by** the steps
- manufacturing carbon anode blocks 2 including stubholes 5,
- lining the stubholes 5 with expanded graphite lining 7,
- placing the anode hanger 3 such that the downwardly facing anode hanger stubs 4 are each extending into a stubhole 5 of the anode 2 and
- fixing the anode hanger 3 to the anode 2 by pouring cast iron 6 into the gap of stubhole 5 formed between the stub 4 and the anode 2

9. Aluminium electrolysis cells containing anode assemblies 1 according to one of the claims 1 to 6.
